

Oct. 4, 1955

W. S. ALLEN

2,719,820

## METHOD FOR COATING STEEL STRIP

Filed Jan. 26, 1951

2 Sheets-Sheet 1



67  
**Inventor:**  
WILLIAM S. ALLEN,  
by: Donald G. Dalton  
his Attorney.

Oct. 4, 1955

W. S. ALLEN

2,719,820

## METHOD FOR COATING STEEL STRIP

Filed Jan. 26, 1951

2 Sheets-Sheet 2



FIG. 3.



*Inventor:*  
WILLIAM S. ALLEN,  
by: Donald S. Dalton  
his Attorney.

1

2,719,820

**METHOD FOR COATING STEEL STRIP**

William S. Allen, Pittsburgh, Pa., assignor to United States Steel Corporation, a corporation of New Jersey

Application January 26, 1951, Serial No. 207,981

4 Claims. (Cl. 204—28)

This invention relates to improved methods and apparatus for coating steel strip with tin or other metals.

Electrolytic methods of tinning sheet steel presently are restricted to coatings of 0.75 pound per base box and under, since hot-dip methods are considered more economical for heavier coatings. Considerable savings could be obtained if hot dip methods could be applied to continuous strip operation, but, even though much effort and experimental development has been devoted to this problem, there has been no satisfactory answer heretofore of which I am aware. The greatest difficulty is the removal of the excess tin that always is applied when the strip passes through a bath of molten tin.

An object of the invention is to provide improved tinning methods and apparatus which are capable of depositing coatings of any desired weight from about 0.5 to 3.0 pounds or heavier per base box on continuous lengths of steel strip.

A further object of the invention is to provide improved tinning methods and apparatus which deposit on steel strip only the amount of tin desired on the finished product.

A further object of the invention is to provide improved coating methods and apparatus which combine electrolytic coating with spray coating to enable a metal coating of any desired weight to be built up on continuous lengths of steel strip.

A further object of the invention is to provide improved apparatus and methods for applying metal coatings to steel strip in which a continuous strip first receives a lightweight prime coating electrolytically and thereafter receives a coating of any desired weight by spraying, the two coatings subsequently being melted into a unified coating alloyed with the steel.

In accomplishing these and other objects of the invention, I have provided improved details of structure, a preferred form of which is shown in the accompanying drawings, in which:

Figure 1 is a side elevational view, in which some details are shown schematically, of a portion of a metal coating apparatus embodying features of the present invention;

Figure 2 is a vertical sectional view of the spray device employed in the apparatus; and

Figure 3 is an end elevational view of the device shown in Figure 2.

Figure 1 shows a portion of a metal coating line which, in accordance with the present invention, includes in combination an electrolytic cell 10 and a spray coating mechanism 12. A continuous steel strip S travels from left to right, passing first through the electrolytic cell and subsequently through the spray coating mechanism. Before reaching the former, the strip is cleaned and pickled in the usual manner. After discharging from the latter, the coated strip can be subjected to any of the usual finishing operations, such as surface chemical treatment and/or oiling.

The electrolytic cell 10 illustrated comprises a tank 13, conductor rolls 14, a sink roll 15 and anodes 16, which

2

in the present example are tin. The tank contains any desired plating bath from which a metal coating, in this instance tin, can be deposited electrolytically on the strip S, as known in the art. Since the electrolytic cell need only deposit only a very lightweight coating on the strip (0.1 to 0.2 pound per base box) only a single cell is sufficient.

Between the electrolytic cell 10 and the spray coating mechanism 12, the strip passes downwardly through a drag-out recovery tank 17, around a sink roll 18 in said tank, upwardly through said tank and through a steam drier 19, over a grounded conductor roll 20 and downwardly through a choke core 21. The strip then passes around two conductor rolls 22 and 23, which are situated at opposite ends of the spray mechanism, hereinafter described, and which introduce alternating current to the strip for melting the coating. The purpose of the choke core is to limit the current which can flow back through the strip from roll 22 and the purpose of the ground on roll 20 is to prevent any of this current from entering the electrolytic cell.

The electrolytic cell 10, the various conductor and sink rolls, the drag-out recovery tank 17, the steam drier 19, and the choke core 21 per se can all be of any standard or desired construction. The various rolls can be power driven for propelling the strip in any usual fashion. The use of alternating current for melting the coating and of the choke core and grounded conductor roll for limiting the flow of such current also is as known in the art. Therefore structural features of these parts and their mode of operation are not described in detail.

The spray coating mechanism comprises an enclosed two-pass muffle 24 which is made of heat insulating material and has an electrically insulated roll 25 in its upper portion. The strip S travels from the conductor roll 22 upwardly through the first pass of the muffle, over the insulated roll 25, downwardly through the second pass of the muffle, and around the conductor roll 23. The muffle has a mechanical seal 26 at its entry end. The conductor roll 23 is mounted in a tank 27 which contains a water or oil bath that both serves as a liquid seal for the exit end of the muffle and also quenches the strip after its coating has melted. The muffle contains a non-oxidizing or reducing atmosphere and the two seals prevent entry of air.

The second pass of the muffle has a section 28 which is of an electrically non-conductive material, such as brick. Two sets of opposed spray nozzles 29 and 29a of non-corrodible material, such as stainless steel, are mounted on opposite sides of the muffle in its section 28. The nozzles of each set can be spaced about 4 inches apart and about 6 to 8 inches from the strip surface. The nozzles are supplied with molten metal, in this instance tin, from individual containers 30 and 30a. Said containers are equipped with burners 31 and 31a which maintain their contents in a molten state. Compressors 32 and 32a supply the nozzles with a stream of non-oxidizing atmosphere from the muffle for atomizing the sprays of molten coating metal. Preferably heaters 33 and 33a are interposed between the compressors and the nozzles to heat the gas before it reaches the latter.

Figures 2 and 3 show the details of a preferred construction of nozzle 29 and container 30, the other nozzle 29a and container 30a being similar. The nozzle contains a needle valve 34 which has an operating solenoid 35. This valve controls the amount of metal sprayed through the nozzle and also furnishes a convenient shut-off. A gas chamber 36 surrounds the nozzle and has a connection 37 for admitting gas from the compressor 32. The container is equipped with a platform 38 and gate 39 for supplying additional bars T of the coating metal.

The spray mechanism can be equipped with electrostatic means for attracting the molten particles of metal

in the spray to the strip. Figure 1 shows two pairs of transformers and electronic rectifiers 40 and 40a, which can be of any standard or desired construction and are connected to low voltage A. C. lines 41 and 42. The rectifiers each have positive and negative D. C. outlet lines 43 and 44. The positive outlet lines 43 are grounded and thus are connected to the strip via the ground. The negative outlet lines 44 are connected to the containers 39 and 39a and to grids 45 and 45a. The output of the rectifiers is at a high voltage, on the order of 100,000 to 150,000 volts. Consequently the particles of molten coating metal and the strip bear opposite electrostatic charges, which cause these particles to be attracted to the strip surface. Optionally the transformers and rectifiers 40 and the grids 45 and 45a can be omitted and the electrostatic charge supplied to the particles of coating metal via the transformers and rectifiers 40a and the spray guns 29 and 29a only. A further possibility is to eliminate the transformers and rectifiers 40a and to supply the electrostatic charges to the particles solely by induction as they pass through the grids 45 and 45a.

The atmosphere within the muffle or else the strip surface, preferably the former, can include a fluxing agent which reduces the surface tension of the particles of coating metal and thus insures a smoother coating. When the furnace atmosphere carries the flux, the flux can be HCl, Cl<sub>2</sub> or SnCl<sub>4</sub> vapor. When the strip carries the flux, the flux can be an aqueous solution of SnCl<sub>2</sub>, or other tin salt, ZnCl<sub>2</sub> or NH<sub>4</sub>Cl or palm oil.

According to the coating method of the present invention, the cleaned and pickled steel strip S traveling at a speed of 100 to 350 feet per minute, passes first through the electrolytic cell 10, where it receives a lightweight prime coating of 0.1 to 0.2 pound per base box. This step per se is performed in the usual manner except that the coating is of lighter weight than when the electrolytically coated strip is a finished product. Next the strip passes through the drag-out recovery tank 17, the steam drier 19, and the choke core 21, all of which perform their usual function. Next the strip passes around the conductor roll 22, through the muffle 24 of the spray coating mechanism 12 and around the conductor roll 23. These two conductor rolls apply alternating current to the strip and heat it electrically sufficiently to melt the metal deposit. This melting also is carried out in the usual manner and the variables are controlled so that the coating attains its melting temperature in the vicinity of the spray nozzles 29 and 29a.

As the strip passes the nozzles, they spray fine particles of molten coating metal on its surface. The opposite electrostatic charges on the particles and on the strip causes these particles to be attracted to the strip surface. The non-oxidizing or reducing atmosphere of the muffle prevents surface oxidation of the particles and the flux enables them to spread uniformly on the strip surface. The weight of coating deposited can be controlled by the opening of the needle valve 34, by adjusting the pressure of gas delivered from the compressors 32 and 32a, and by adjusting the strip speed. For example at a line speed of 300 feet per minute and a tin coating of 1.5 pounds per base box, nozzles spaced 4 inches apart would be required to spray about 0.4 pound of tin per minute.

About the time the strip passes the nozzles, the coating melts throughout and alloys itself with the steel surface of the strip. The strip then enters the quenching liquid in tank 27 and the coating again solidifies. The coated steel strip then is ready for any desired finishing steps.

The method of the present invention is intended primarily for tinning, but it also can be used for applying coatings of lead, terne, zinc and other metals. It is also possible to apply coatings in which the electrolytic prime coat is a different metal from the sprayed coating. By choosing the prime coat so that it is capable of alloying with both the steel and the sprayed coating, it serves both as a bonding agent and insulator between the steel surface and the outer coating. Thus a coating, the outer surface of which is predominantly lead, could be made by spraying molten lead on a thin electrolytic tin prime coat and then melting. Or a zinc coating having a thin, more flexible alloy than conventional galvanized coatings, would result from spraying molten zinc on a similar tin coat and melting.

From the foregoing description, it is seen that the present invention affords a simple and effective apparatus and method for tinning or otherwise coating continuous steel strip in which the coatings can be of any desired weight. The method and apparatus attains all the advantages inherent in continuous strip coating, not possible previously when heavy coatings were required. The conventional flux pot with its corrosive and toxic fumes is eliminated. The grease pot also is eliminated, thus greatly simplifying cooling and cleaning problems.

While I have shown and described certain preferred embodiments of the invention, it is apparent that modifications may arise. Therefore, I do not wish to be limited to the disclosure set forth but only by the scope of the appended claims.

I claim:

1. A method of applying to steel strip coatings of metals of the group consisting of tin, terne, lead and zinc comprising electrolytically applying to the strip a lightweight prime coating of one of said metals, said prime coating being of a weight equivalent to 0.1 to 0.2 pound per base box, introducing the strip to a sealed enclosure having a non-oxidizing atmosphere, spraying a heavier coating of one of said metals on the strip within said enclosure, heating the strip within said enclosure and controlling the heating so that the strip surface attains a temperature sufficient to melt the prime coating and alloy the coatings with the strip surface in the vicinity of the point where the heavier coating is sprayed thereon, and quenching the strip.
2. A method as defined in claim 1 in which the metal used in both coatings is tin.
3. A method as defined in claim 1 in which the heavier coating is sprayed on the strip in an electrostatic field.
4. A method as defined in claim 1 in which the strip is heated electrically.

References Cited in the file of this patent

UNITED STATES PATENTS

|    |           |               |                |
|----|-----------|---------------|----------------|
| 55 | 1,517,910 | Kirschner     | Dec. 2, 1924   |
|    | 2,048,552 | Johnson       | July 21, 1936  |
|    | 2,159,297 | Shover        | May 23, 1939   |
|    | 2,282,022 | Bishop et al. | May 5, 1942    |
|    | 2,304,709 | Rubin         | Dec. 8, 1942   |
|    | 2,358,104 | Scavullo      | Sept. 12, 1944 |
|    | 2,414,923 | Batcheller    | Jan. 28, 1947  |
|    | 2,505,530 | Davis         | Apr. 25, 1950  |
|    | 2,551,035 | Miller        | May 1, 1951    |
|    | 2,566,468 | Taylerson     | Sept. 4, 1951  |

FOREIGN PATENTS

|         |               |               |
|---------|---------------|---------------|
| 196,695 | Great Britain | Apr. 27, 1923 |
|---------|---------------|---------------|